

Patented July 5, 1927.

1,634,527

# UNITED STATES PATENT OFFICE.

WILLIAM H. WOOD, OF SOUTH EUCLID, OHIO.

## STORAGE BATTERY.

No Drawing.

Application filed October 15, 1924. Serial No. 743,844.

This invention relates to storage batteries and has for its objects the provision of a lead type battery of decreased internal resistance thereby producing a higher discharge rate 5 and a larger effective voltage especially in the cold, thereby enabling superior performance under severe conditions such as cranking internal combustion engines in winter weather which in turn enables the 10 use of a smaller, lighter and cheaper battery to do the same work. Another object of the invention is the provision of an improved separator which can be sold and shipped in bone dry form, either alone or as constituting a part of an assembled battery. Other 15 objects and advantages of the invention will become apparent as the description proceeds.

Accumulators of the lead type as employed for vehicle use consist of spaced positive and negative plates and thin wooden separators between them. Nearly every kind of wood has at different times been employed for this purpose, the preferred species at the present time being generally cedar, red- 20 wood, and quarter-sawed oak. Many of these are treated with lye to remove the resinous and acid portions which might be deleterious to the battery elements. This treatment, however, leaves the cellulose in- 25 tact, indeed it has to some extent the effect of "mercerizing" it, with the result that upon the slightest drying the cellulose fibers contract and close up the pores in such a way as greatly to injure the performance of any 30 battery made therefrom.

According to my invention a part of this cellulose is removed by the action of sulphuric acid of the proper strength. The strength of the acid and the duration of 40 treatment thereby depends upon the species of the wood and the previous treatment if any to which it has been subjected. If separators are used which have already been treated with lye, a weaker acid, and a shorter 45 time of treatment are required because the alkali treatment has already removed a considerable part of the resinous substances so that the acid can get more immediate action on the cellulose. As an example of a bene- 50 ficial treatment I instance soaking for fifteen minutes in a solution of sulphuric acid in water of a specific quantity of 1.400. In case of quarter sawed oak I instance as a good treatment the immersion for one-half hour 55 in a similar solution. This treatment is also beneficial to other types of wood which do

not ordinarily make very good separators such as plain-sawed oak and other hard woods. Of course the time of treatment also depends upon the strength of the acid and the temperature, and I do not limit myself in either respect although I have discovered that 1.300 is too low and 1.500 is too high for practical production conditions. 60

If the separators are taken from this acid treatment and assembled immediately in the final battery its discharge rate and available voltage are substantially increased. In case it is impossible to assemble the separators immediately in a battery, as is usually the 70 case under large scale production conditions, it is necessary to observe certain precautions to avoid injury by continued action of the acid, which action may even be intensified by concentration due to evaporation. Mere 75 rinsing in water is sufficient for a delay of a few minutes but not for any long interval since the acid in the pores cannot be wholly removed in this manner, and upon evaporation will become so concentrated as in time 80 to injure the material. If kept submerged in water (or a weaker sulphuric acid solution) these treated separators can be kept indefinitely.

However, it is possible by immersing these 85 separators in a hot concentrated solution of Epsom salts to render the separators immune to drying and to the evils of shrinkage or undue corrosion. Prior to immersion these 90 separators ought to be rinsed with water to an extent sufficient at least to remove the adherent acid. The concentration and temperature of the solution can vary considerably, but I prefer such conditions that the 95 separators will be sensibly dry as soon as they reach air temperature, although I do not limit myself even to this as I have had excellent results by the use of cold solutions. It is only necessary to leave the separators in the solution until they are thoroughly 100 impregnated, but the stronger the solution the quicker the separator will become dry after removal.

It is of course possible to remove the sulphuric acid by the use of steam, formaldehyde, etc., but even in this case it is very advantageous to employ the Epsom salt treatment in order to prevent the shrinkage and loss of porosity which would otherwise occur. Removal of the acid is not necessary, 110 however, in case of the Epsom salt treatment.

I do not restrict myself to the treatment of separators wherein cellulose occurs naturally, as I have found it valuable in connection with devices of this character where-  
5 in the cellulose is introduced artificially, as by embedding cotton, sawdust, etc, in a matrix of rubber. The presence of Epsom salts is not injurious to a lead accumulator and it is not necessary to wash or soak the  
10 separators or otherwise cleanse them before assembling in battery form in case the separators are treated and used at different times or places, or before adding electrolyte to the jars in case these be used in making  
15 bone dry assemblies, either charged or uncharged. Accordingly I do not limit myself except as set forth in my several claims, which I desire may be construed each independently of the limitations contained in  
20 other claims.

Having thus described my invention what I claim is:

1. The process of treating the wood separators of lead accumulators which contains  
25 the step of immersing them in sulphuric acid of a specific gravity above 1.300 and below 1.500 until sufficient cellulose is removed therefrom to increase the porosity sensibly, but without disintegration of the organic  
30 structure and afterward reducing the concentration of the adherent acid.

2. The process of treating the wood separators of lead accumulators which contains the step of removing out of them a portion  
35 of their cellulose by treatment with sulphuric acid of specific gravity above 1.300.

3. The process of treating the separators of lead accumulators which contains the step

of immersing them in sulphuric acid of a specific gravity above 1.300 and below 1.500 40 until sufficient cellulose is removed therefrom to increase the porosity sensibly, and afterward immersing in a strong solution of Epsom salts.

4. The process of treating the wood separators of lead accumulators which contains the step of removing out of them a portion of thin cellulose by treatment with sulphuric acid of specific gravity above 1.300 and afterward impregnating with Epsom salts. 45

5. A separator for storage batteries consisting essentially of a thin plate rendered porous by the presence of organized cellulose, the pores of the plate being filled with sulphuric acid, water, and Epsom salts. 50

6. A separator element for storage batteries consisting of a sheet of porous wood impregnated with sulphuric acid and magnesium sulphate. 55

7. The process of arresting the corrosive action of sulphuric acid on the elements of a storage battery which consists of washing off the externally adherent acid and soaking the element in a strong solution of magnesium sulphate. 60

8. The process of improving the porosity of a battery separator containing organized cellulose which contains the steps of first removing a part of the cellulose with a strong solution of sulphuric acid, and then arresting the action of the sulphuric acid with a strong solution of Epsom salts. 65

In testimony whereof, I hereunto affix my signature.

WILLIAM H. WOOD.